

# UNITED STATES PATENT OFFICE.

GEORGE W. PRENTICE, OF PROVIDENCE, RHODE ISLAND.

## FABRIC FOR LACING-TIPS AND THE LIKE AND COMPOSITION FOR THE SAME.

939,313.

Specification of Letters Patent. Patented Nov. 9, 1909.

No Drawing.

Application filed August 18, 1906. Serial No. 331,184.

*To all whom it may concern:*

Be it known that I, GEORGE W. PRENTICE, of Providence, in the county of Providence and State of Rhode Island, have invented 5 certain new and useful Improvements in Fabrics for Lacing-Tips and the Like and Compositions for the Same; and I do hereby declare the following specification to be a full, clear, and exact description thereof.

10 The object of the invention is to produce a fabric especially adapted for use in making fabric tips for lacings, such as shoe-lacings and the like, in place of the metal tips heretofore employed. For such use it is desirable that the fabric shall possess certain peculiar characteristics. Thus the fabric, which should be provided with an adhesive substance for securing the tip to the lacing proper, must be comparatively stiff, 15 in order that the finished lacing tip may possess the necessary strength and rigidity. On the other hand the fabric must be sufficiently pliable or flexible to enable the fabric to be readily bent or wrapped around 20 the body of the lacing without breaking or cracking. So also, while the fabric should be provided with an adhesive substance, it is desirable that the fabric should be rendered substantially non-adhesive for 25 purposes of handling, but should at the same time be capable of being readily made adhesive when it is to be applied to the lacing. It is further desirable that the fabric should 30 be comparatively water-proof and should also be of such a character that the lacing tip when finished will be smooth and even and have what may be termed a satin-like 35 appearance.

For the production of a fabric possessing 40 these several characteristics the invention consists in treating a textile fabric, preferably a woven cotton fabric such as cambric or canvas, with a composition containing the following ingredients, viz., ordinary 45 glue, fish-glue or isinglass, and lamp-black, and in the fabric or article of manufacture so produced.

For securing the best results the proportions of the several ingredients above named 50 should be substantially as follows: 30 parts of glue; 30 parts of isinglass; and 10 parts of lamp-black. It will be understood, however, that the invention is not limited to the 55 employment of the exact proportions above named, but that the same may be varied without departing from the invention. Of

the ingredients named the glue constitutes the main adhesive substance in the composition, while the isinglass, which is likewise adhesive, serves to give to the composition 60 and to the fabric to which it is applied the requisite pliability and flexibility, and also serves to render the fabric comparatively water-proof. If the glue alone were used without the isinglass, the composition and 65 the fabric to which it is applied would be too hard and brittle, and the fabric would be likely to crack or split in bending or wrapping the same upon the lacing. The presence of the isinglass in the composition prevents 70 such cracking or splitting of the fabric. The lamp-black serves to give color and body to the composition and constitutes a sizing for the fabric when the composition has been applied thereto which serves to render the 75 fabric non-adhesive except upon the application of moisture.

The composition above described will be black and the fabric with the composition applied thereto will be suitable to apply to 80 the ordinary black lacings. If the fabric is to be employed for tips for lacings of other colors, suitable coloring matter may be added to give to the composition a color like or 85 similar to that of the lacings.

In preparing the composition the several ingredients are put in liquid form, the glue and the isinglass being dissolved with water, and the lamp-black being mixed with alcohol, preferably with the aid of heat in each case. The ingredients are then thoroughly 90 mixed together, heat being also preferably applied during the mixing process to maintain the ingredients in liquid form. As the lamp-black, by reason of the presence of the alcohol, has a tendency to rise to the top and thus to separate from the glue and isinglass, it is desirable that the composition should be applied to the fabric as promptly as possible 95 after the ingredients have been mixed together. It has been found in practice, however, that, even if the composition stands for a sufficient length of time to enable the lamp-black to separate more or less from the other ingredients, the result of the application of 100 the composition to the fabric is substantially the same as when the composition is applied directly after the mixing of the ingredients. It is further found that in either case a sufficient quantity of the lamp-black remains 105 at or near the surface of the fabric to constitute a sizing and thereby render such sur-

face substantially non-adhesive except upon the application of moisture.

The composition may be applied to the fabric in any suitable manner, such as by 5 dipping or immersing the fabric in the liquid composition. A convenient way will be to draw the fabric through a vessel containing a suitable quantity of the composition, and preferably the vessel is provided with a 10 guide-bar near the bottom of the vessel around which the fabric may be passed, and so that the fabric may be drawn first downward and then upward through the composition.

15 With respect to the proportions of the ingredients it is to be understood that the proportions above named are the proportions of the ingredients in their dry and solid condition and before they have been dissolved 20 in water and alcohol respectively. The quantities of water and alcohol employed will be determined by the consistency of the composition desired, and this consistency may be varied to a considerable degree 25 according to the judgment of the user.

After the composition has been applied to the fabric, the fabric is to be dried in any suitable manner. It is preferred, when the 30 fabric has been partially dried, to pass the treated fabric between pressure rollers, which serves to give to the fabric a smooth and finished surface.

It will be found that a fabric treated with a composition substantially such as above 35 described possesses the peculiar qualities above referred to. Thus the fabric has a certain amount of stiffness or rigidity, while at the same time it is sufficiently pliable or flexible to be bent or wrapped around the 40 body of a lacing without breaking or cracking. The fabric also has a considerable body, and although provided with a considerable quantity of adhesive substance is nevertheless non-adhesive in its finished condition 45 and may be handled freely without any sticking to the fingers. At the same time by the application of a slight amount of moisture the fabric becomes distinctly sticky and adhesive. It will be further 50 found that this adhesive quality continues

only so long as the moisture remains, and that as soon as the moisture has evaporated the fabric is again non-adhesive, although capable of being again rendered adhesive by the application of moisture thereto. Certain 55 additional results and advantages may be obtained by adding shellac to the ingredients above named in forming the composition. In such case a proper quantity of shellac to be employed in connection with the proportions of the other ingredients named will be 30 parts of shellac in its dry form. This dry shellac is to be dissolved in alcohol, preferably with the aid of heat, as in the case of the lamp-black, and the 60 shellac in liquid form is to be thoroughly mixed with the other ingredients. The shellac when employed will serve to facilitate the drying of the fabric after being treated with the composition, and with the lamp- 70 black will act as a sizing. The shellac will also serve to increase the water-proof quality of the fabric, and also to increase the rigidity of the finished tip and the satin-like appearance thereof. 75

Preferably the fabric is treated in large pieces as it comes from the loom, and is then cut into strips of a width equal to the length of lacing tip desired, the several tips of proper size being then cut from these strips. 80

What I claim as my invention and desire to secure by Letters Patent is:

1. As an article of manufacture a textile fabric treated with a composition of glue, isinglass, and lamp-black, substantially as 85 described.

2. A composition for treating textile fabrics composed of glue, isinglass, and lamp-black, substantially as described.

3. As an article of manufacture a textile 90 fabric treated with a composition of glue, isinglass, shellac, and lamp-black, substantially as described.

4. A composition for treating textile fabrics composed of glue, isinglass, shellac, and 95 lamp-black, substantially as described.

GEORGE W. PRENTICE.

Witnesses:

W. H. THURSTON,

J. H. THURSTON.